

## UNITED STATES PATENT OFFICE

2,347,217

## LUBRICATING COMPOSITION

Carl F. Prutton, Cleveland, and Albert K. Smith, Shaker Heights, Ohio, assignors, by mesne assignments, to The Lubri-Zol Development Corporation, Cleveland, Ohio, a corporation of Delaware

No Drawing. Application December 19, 1940,  
Serial No. 370,838

4 Claims. (Cl. 252—48)

This invention relates, as indicated, to lubricating compositions and more particularly, to compositions for use in connection with the lubrication of the working parts of internal combustion engines, motor vehicles, etc. and it is among the objects of the invention to provide compositions obviating the disadvantages of the usual petroleum oils.

It has been explained by specialists in this particular field of the art that a lubricant employed for the purpose of reducing friction between relatively movable metallic parts functions in two ways commonly referred to as "thick-film" lubrication and "thin-film" lubrication.

In "thick-film" lubrication the bearing surfaces are completely separated by a relatively thick continuous film of the lubricating composition employed. When friction between the moving parts is measured in this case, the results obtained are independent of all factors except pressure, speed and the viscosity of the lubricating composition. A single curve representing all data may be found by plotting the coefficient of friction against a particular function consisting of the product of the viscosity of the lubricating composition and the speed of relative movement of the parts divided by the pressure per unit area of the bearing surface, as long as the value of such function is greater than a definite amount. At this minimum point, reduction of viscosity or speed or an increase in the pressure results in a breaking down of the film of lubricant. Although the value of the coefficient of friction is lowest at the point at which the film is about to break down, the increase in the coefficient for higher viscosity and speed or lower pressure is relatively slight. The conditions resulting in "thick-film" lubrication are, therefore, those which result in low friction.

For pressures sufficiently great or for correspondingly low values of viscosity or speed, the film of lubricant, as above indicated, is broken down and if it is not entirely destroyed, the metallic bearing surfaces are still affected to some extent, at least by the presence of the lubricating composition. This condition is commonly referred to as "thin-film" lubrication.

When one of the bearing surfaces is a metal such as bronze or babbitt, seizure does not take place at once but the coefficient of friction increases rapidly to abnormally high values with each slight further increase in pressure or decrease in viscosity or speed. For a given set of bearings the data obtained for "thin-film" lubrication may be approximately coordinated into a single curve but only on plotting coefficient of friction against the product of viscosity and speed divided by the square root of the pressure.

If both bearing surfaces are of steel, seizure or scoring will result almost immediately upon failure of "thick-film" lubrication when a pure mineral oil is the sole lubricating composition employed.

It is among the objects of our invention to provide a lubricating composition which may be employed to reduce the friction between relatively movable metallic surfaces under pressures and other factors which result in what has been above explained as "thick-film" lubrication and a composition which may be employed for such "thin-film" lubrication and without a material increase in the coefficient of friction between the parts over that found during "thick-film" lubrication.

Other objects of our invention will appear as the description proceeds.

To the accomplishment of the foregoing and related ends, said invention, then, consists of the means hereinafter fully described and particularly pointed out in the claims.

The following description sets forth in detail one approved combination of ingredients embodying our invention, such disclosed means constituting, however, but one of various forms in which the principle of the invention may be used.

Broadly stated, this invention comprises incorporating certain forms of halogenated carbon compounds with certain types of oil bases. More specifically, the invention comprises incorporating a halogenated carbon compound with a sulphur treated oil base.

By the term "sulphur treated oil" as employed in this description, is meant any suitable oil base which has been treated with sulphur, for example, the composition produced by heating sulphur with a fixed oil, such as lard oil or fish oil; or to which sulphur or a sulphur compound, (e. g. di-phenyl di-sulphide) has been added, so that a certain amount of sulphur is present in active or loosely combined form. It has been found that a suitable oil base containing from 0.50% to 2.50% of sulphur in active or loosely combined form is best suited for use in a composition according to the present invention. These percentages are not to be construed, however, as limitations but merely an indication of the range of sulphur in the form defined for optimum results.

Examples of other sulphur compounds which may be added to an oil base to obtain a sulphur treated oil are the products obtained by the reaction of an organic halogen compound with a sulphur compound, such as for example the inorganic sulphides and polysulphides, resulting in the complete or partial substitution of a sulphur-bearing radicle for the halogen. Examples of

such materials are the reaction products of sodium sulphide, sodium polysulphide, sodium thiocyanate, or potassium xanthate with aralkyl chlorides such as:

Benzyl chloride  
Chlor-benzyl chlorides  
Xylyl chloride  
Chlor-xylyl chlorides

or with alkyl chlorides such as:

Lauryl chloride  
Cetyl chloride  
Chlorinated petroleum naphtha  
Chlorinated petroleum wax

or with cyclo-aliphatic chlorides such as:

Cyclohexyl-methyl chloride  
Naphthyl chloride

The halogenated carbon compounds which are added to sulphur-treated oil bases, as above defined, in accordance with the present invention, are preferably halogenated or more specifically chlorinated carbon ring compounds and preferably oxygen-containing halogenated, or more specifically, chlorinated carbon ring compounds.

The halogenated oxygen-containing carbon ring compounds added to a sulphur treated oil base are, as above indicated, preferably of the chlorinated species and particularly the following compounds have been found to produce very satisfactory results, viz: halogenated or more specifically, chlorinated oxygen-containing substituted benzene compounds such as:

Chlorinated phenols  
Chlorinated cresols  
Chlorinated diphenylether  
Chlorinated methyl salicylate

halogenated substituted di-phenyl such as:

Chlorinated P-phenyl phenol  
Chlorinated di-xenyl ether

chlorinated substituted naphthalenes such as:

Chlorinated naphthols;

as well as the aromatic ethers, phenols, acids, the esters and the aldehydes.

For many purposes it is particularly advantageous to use a halogenated oxygen-containing carbon-ring compound which contains a carbonyl

(>C=O)

radicle such as the cyclo-aliphatic and aromatic aldehydes, amides, ketones, acids, esters and salts, thio-acids and esters and salts of thio-acids.

Specific examples of preferred compounds of which the halogen-bearing derivatives may be used for our purpose are as follows:

Aldehydes:

Benzaldehyde  
Furfural  
Phenyl acetaldehyde  
Lauryl benzaldehyde

Amides:

Acetanilide  
Anilides of naphthenic acids  
Benzamide  
Benzanilide  
Lauryl benzamides  
Lauryl benzanilides  
Naphthyl benzamides  
Naphthyl benzanilides  
Stearanilide

Ketones:

Acetophenone  
Anthraquinone  
Benzaphenone  
Benzil  
Benzoin  
Butyl benzophenones  
Camphor  
Cyclohexanone  
Di(methyl-phenyl) ketone  
Dinaphthyl ketone  
Dixenyl ketone  
Furil  
Furoin  
Lauryl benzophenones  
Methyl benzophenones  
Methyl xenyl ketone  
Naphthyl benzene  
Naphthyl diphenyls  
Naphthyl naphthalenes  
Stearoyl benzene  
Stearoyl naphthalenes  
Stearoyl diphenyls  
Stearoyl diphenyl ethers  
Phenyl naphthyl ketone

Acids:

Azobenzoic acid  
Azolauryl benzoic acid  
Benzene sulphonic acid  
Benzoic acid  
Cinnamic acid  
Diphenyl acetic acid  
Ethyl salicylic acid  
Mercapto benzoic acid  
Mercapto lauryl benzoic acids  
Mercapto rosolic acid  
Lauryl benzene sulfonic acids  
Lauryl benzoic acids  
Lauryl phenyl acetic acids  
Lauryl phenyl propionic acids  
Lauryl salicylic acids  
Lauryl thiobenzoic acids  
Lauryl toluic acids  
Naphthyl benzene sulfonic acids  
Naphthyl benzoic acids  
Naphthyl phenyl acetic acids  
Naphthyl salicylic acids  
Naphthyl thiobenzoic acids  
Naphthyl toluic acids  
Phenoxyphenyl stearic acid  
Phenyl acetic acid  
Phenyl mercapto stearic acid  
Phenyl propionic acid  
Phenyl stearic acid  
Stearoyl benzene sulfonic acid  
Stearoyl benzoic acids  
Stearoyl phenyl acetic acids  
Stearoyl salicylic acids  
Stearoyl thiobenzoic acids  
Stearoyl toluic acids  
Thiobenzoic acid  
Toluic acid

Esters:

65 Amyl salicylate  
Benzyl acetate  
Benzyl benzoate  
Benzyl stearate  
Butyl azobenzoate  
70 Butyl esters of pyrrole carboxylic acid  
Butyl esters of thiophene carboxylic acid  
Butyl benzoate  
Butyl thio-benzoate  
75 Butyl ester of mercapto rosolic acid  
Butyl ester of phenyl acetic acid

## Esters—Continued

Butyl ester of phenyl stearic acid  
 Butyl furoate  
 Butyl mercapto benzoate  
 Butyl toluate  
 Dilauryl phthalate  
 Dibutyl phthalate  
 Esters of cinnamic acid  
 Esters of diphenyl acetic acid  
 Ethyl ester of phenyl acetic acid  
 Esters of ethyl salicylic acid  
 Ethyl toluate  
 Esters of phenyl mercapto stearic acid  
 Esters of phenyl propionic acid  
 Lauryl benzoate  
 Lauryl salicylate  
 Lauryl toluate  
 Lauryl ester of phenyl acetic acid  
 Methyl ester of lauryl salicylic acid  
 Methyl ester of phenyl stearic acid  
 Methyl ester of phenyl mercapto stearic acid  
 Methyl ester of naphthenyl benzoic acid  
 Methyl ester of stearoyl benzoic acid  
 Lauryl ester of phenyl propionic acid  
 Methyl toluate  
 Phenyl acetate  
 Phenyl benzoate  
 Phenyl stearate  
 Salts of organic bases:  
 Aniline oleate  
 Aniline stearate  
 Benzylamine stearate  
 Dilauryl amine benzoate  
 Dilauryl amine salt of phenyl stearic acid  
 Lauryl-pyridine stearate  
 Lauryl-quinoline stearate  
 N-lauryl aniline oleate  
 N-lauryl aniline stearate  
 N-lauryl aniline mercapto stearate  
 N-lauryl aniline naphthenate  
 N-lauryl naphthylamine stearate  
 N-naphthenyl aniline stearate  
 N-naphthenyl butylamine benzoate

## Salts of inorganic bases:

Aluminum phenyl mercaptostearate  
 Aluminum phenyl stearate  
 Barium phenyl stearate  
 Calcium lauryl thiobenzoate  
 Calcium naphthenyl benzoate  
 Calcium naphthenyl thiobenzoate  
 Calcium phenyl mercapto stearate  
 Calcium phenyl stearate  
 Calcium phenyl thiostearate  
 Calcium stearoyl benzoate  
 Calcium stearoyl thiobenzoate  
 Sodium phenyl mercaptostearate  
 Sodium phenyl stearate  
 Zinc naphthenyl benzoate

The "halogen derivatives" referred to above may be prepared by (a) directly halogenating (e. g. chlorinating) the compounds listed, or by (b) treating the compounds listed with a halogenating agent (e. g.  $\text{SOCl}_2$ ,  $\text{PCl}_5$ , etc.) or by (c) the reaction of halogen-containing intermediates. For example, halogen derivatives of methyl salicylate may be prepared by

(a) direct halogenation of methyl salicylate, e. g. by passing chlorine through methyl salicylate preferably in the presence of a catalyst such as iodine,  $\text{PCl}_3$ , iron, etc., or by  
 (b) treating methyl salicylate with  $\text{PCl}_5$ , or by  
 (c) esterifying chlor-salicylic acid with methyl alcohol.

By the term "naphthenyl" as used herein, we mean the radicles which have the structure



5 (in which R is a cyclo-aliphatic group, or an alkyl-cyclo-aliphatic group) which result from naphthenic acids by the removal of the hydroxyl group. For example, "naphthenyl" chloride 10 would be the acid chloride derived from a naphthenic acid and "naphthenyl benzene" would be the compound resulting from the Friedel-Crafts condensation of naphthenyl chloride with benzene.

15 Since generally the addition of compounds of the class including the above enumerated reduce the viscosity of the oil base to which the same are added, if a large percentage of such compounds are added, there will be a tendency to 20 destroy "thick-film" lubrication because of such reduction in viscosity. If an excessive quantity of such compounds are added, all of the lubrication will then be of the "thin-film" type and therefore produce a decided increase in the amount of friction developed.

25 Optimum results are obtained by using minimum quantities of these halogenated compounds so that their beneficial effect in the region of "thin-film" lubrication will not be over-shadowed 30 by their detrimental effect in the region of "thick-film" lubrication.

Our invention contemplates incorporating with a sulphur treated oil base a total of less than 20% of at least one halogenated oxygen containing 35 carbon ring compound of the enumerated class.

35 The optimum amount of the halogenated compound to be employed will depend largely upon the halogen content of the particular compound, its physical characteristics and especially its effect 40 on the viscosity of the oil to which it is added. The particular use for which the lubricant is intended is also a governing factor in determining the amount of the compound to be added.

For the purpose of lubricating and reducing the 45 friction between the relatively movable parts of an internal combustion engine such as crank case bearings, piston and cylinder surfaces, as well as piston rings and valves, a composition according to our invention comprises a large proportion of 50 a sulphur treated oil base and concentrations of from one-half to two per cent of halogenated compounds of the above class containing from 50% to 25% of chlorine. If the valve structure of the engine is to be lubricated separately from 55 the remainder of the mechanism or by means acting in an auxiliary fashion, the composition for such purposes will preferably contain a larger amount of such halogenated compounds, i. e., from 2% to 10%.

60 The limit of the amount of the halogenated compounds which may be added to a sulphur treated oil base and which will produce improved results depends, as above indicated, upon the reduction in viscosity of the composition caused by 65 the addition of such compounds. Certain of the more viscous compounds, for example, dimethyl dichlor benzophenone, may be added in amounts exceeding 10% without causing too great a reduction of viscosity. In any event, the resultant 70 composition will have inferior lubricating properties if the loss of viscosity is too great as will result from the use of more than 20% of halogenated compounds of any type.

75 It has been found that for optimum results a certain relationship should be maintained be-

tween the amount of chlorine and the amount of sulphur, when the halogenated compounds of the above class are added to a sulphur treated oil. It has been found that to an oil base having a low content of sulphur in active or loosely combined form, halogenated compounds should be added in correspondingly low concentrations for best results.

When the halogenated compounds of the above class added to the sulphur treated oil base are of the closed ring type in contradistinction to the open chain type, certain advantages are obtained which may be briefly explained as follows:

In case of oil in actual use in machinery of any kind and particularly in the crank case of internal combustion engines, moisture is usually present to some extent and due to condensation may even accumulate to form a separate layer. There is usually sufficient water present, therefore, for hydrolysis to take place, particularly when the addition of a chlorinated compound is made to the extent of only a few percent.

Experiments have shown that when compounds which readily hydrolyze, such as chlorinated open chain compounds, are added to the sulphur treated oil base, hydrolysis may take place to such an extent that the metal parts of any machine being lubricated will be seriously attacked and corroded by the acid generated. On the other hand, the addition of chlorinated carbon ring compounds of the above enumerated class does not cause corrosion, particularly when such compounds are of the type in which the halogen is directly attached to a benzenoid ring.

The oil base of our lubricating compositions is a lubricating oil of the type best suited for the particular use for which the ultimate composition is designed. When the lubricating compositions of our invention are designed for the lubrication of automobiles, the oil base will of course preferably consist of a refined mineral lubricating oil of lubricating viscosity for the particular point of application. In other words, the conventional gear oil may be used for the lubrication of gears, for example, mineral oil having a viscosity range of from an S. A. E. 80 to an S. A. E. 140. Generally a lighter, more highly refined oil may be used in the crank case, such as a motor oil having a viscosity range of from an S. A. E. 10 to an S. A. E. 50.

This invention is applicable to lubricating compositions in which the base may consist either entirely or in part of synthetic oils, hydrogenated oils, and volatilized oils.

The oil base may also desirably contain other well known constituents such as those which improve the oiliness, pour point, cold test, and oxidation properties, etc., of the oil. In general compositions of our invention may be employed with any commercially available addition agents for the above defined purposes since they are generally compatible with the same in the amounts usually used.

The composition comprising our invention has certain advantages when used as a lubricant of which the following may be mentioned:

First: By the use of this composition it is possible to extend the pressure range between the bearing surfaces because of the reduced tendency for bearing surfaces so lubricated to become scored or to seize at higher pressures than are allowable with ordinary lubricants.

Second: The friction between the bearing surfaces is reduced, especially in the higher pres-

sure range below that obtained with ordinary lubricants.

When used in conjunction with a hydrocarbon lubricating oil, it is obvious that, generally, only such amounts of the addition agent may be included as are soluble in the specified amount of oil. By the term "soluble," as herein used, it is intended to indicate the ability to form not only true solutions but also any form of substantially permanently homogeneous composition when incorporated in mineral oil. With most of the compounds there is usually little difficulty, especially if the incorporation is effected in the manner described in Cornell Patent No. 2,042,880, and since quite small percentages often give remarkably improved results, it is seldom of extreme importance that the addition agents be oil-soluble in all proportions.

The addition agents above enumerated for use in my compounded lubricants include certain ones which may be found to at least partially decompose under conditions of extreme stress such as the very high temperature encountered in certain classes of use, while others are quite stable even under such extreme conditions.

The use for which the lubricant is designed therefore determines the particular type of addition agent to be selected. A certain amount of decomposition, which proceeds at a relatively slow rate, is usually not harmful. Care should be exercised, however, to select for a particular set of operating conditions, an addition agent which in the oil base used will not decompose under such operating conditions except at a low rate.

By the term "stable" as used herein in describing the addition agents is meant the characteristics of the addition agents which enables them to resist decomposition in the oil under the condition of use for which the lubricating composition is designed.

In view of the particular uses for which my compounded lubricants are intended, it is apparent that of the materials included in the foregoing enumeration of the addition agents which may be employed, those which are readily oil-soluble are the ones preferred for use. When these compounded oils are designed for use under conditions where high temperatures are usually encountered, the addition agents should be stable at elevated temperatures. For use in crankcase lubricants for internal combustion engines, they should preferably be stable to the extent where there will be substantially no decomposition, when the lubricating composition is exposed to temperatures up to 250° F.

With regard to the use of sulphur treated oil in combination with halogenated compounds, it should be noted that for sufficiently desirable results, the major proportion of the ultimate composition need not consist entirely of sulphur-treated oil, but a suitable oil base such as mineral oil may have added thereto minor quantities or proportions of either a sulphur treated oil or a sulphur compound, and a halogenated compound.

This application is a continuation in part of copending application Serial No. 744,600, filed September 17, 1934, which was in turn a continuation of application Serial No. 649,734, filed December 31, 1932, now Patent No. 2,213,532, and application Serial No. 170,500, filed October 22, 1937, now Patent No. 2,204,620 (a division of application Serial No. 737,070, filed July 26, 1934). Other modes of applying the principle of the

invention may be employed, change being made as regards the details described, provided the features stated in any of the following claims or the equivalent of such be employed.

We therefore particularly point out and distinctly claim as our invention:

1. A lubricating composition comprising a major proportion of mineral lubricating oil and minor amounts of both a sulphur treated oil and a stable oil-soluble halogen bearing organic ring compound containing a carbonyl radicle.

2. A lubricating composition comprising a major proportion of mineral lubricating oil and

minor amounts of both a sulphur treated oil and a stable oil-soluble halogen bearing aromatic compound containing a carbonyl radicle.

3. A lubricating composition comprising a major proportion of mineral oil and minor amounts of both a sulphur treated oil and a halogen-bearing methyl salicylate.

4. A lubricating composition comprising a major proportion of mineral oil and minor amounts of both a sulphur treated oil and chlor-methyl salicylate.

CARL F. PRUTTON.  
ALBERT K. SMITH.